

Feb. 17, 1931.

J. W. COWELL

1,793,437

WALL BOARD ENAMEL AND METHOD OF APPLYING THE SAME

Filed Dec. 16, 1927



Fig. 1.



Fig. 2.



Fig. 3.



Fig. 4.

Inventor:

John W. Cowell

By *Milo B. Stevens Co.*

Attorneys

## UNITED STATES PATENT OFFICE

JOHN W. COWELL, OF GRAYLING, MICHIGAN

## WALL-BOARD ENAMEL AND METHOD OF APPLYING THE SAME

Application filed December 16, 1927. Serial No. 240,475.

My invention relates to protective coatings for wallboard and like sheet materials, and my main object is to produce a coating of this kind in the nature of an enamel of a durable 5 character.

A further object of the invention is to produce an enamel which produces a hard and vitreous finish, which is waterproof and can stand hard usage.

10 A still further object of the invention is to lend the novel enamel a degree of flexibility which will resist cracking or checking as the wallboard is handled, cut or nailed.

15 Another object of the invention is to compound the novel enamel in a manner to permit of its preparation in various colors and imitations of stone, graining, marble veining and other effects.

20 A final but nevertheless important object of the invention is to apply the novel enamel by a unique method, whereby to assure the perfect coating of the same upon the wallboard.

25 With the above objects in view and any others that may suggest themselves in the specification and claims to follow, the composition of the novel enamel will first be treated, reference being later made to the accompanying drawing in which the method 30 of applying the enamel to the wallboard is illustrated.

To compound the enamel, I provide the following ingredients: Magnesite, 1 part by volume; finely divided silica, 1 part by volume; finely divided asbestos, 1 part by volume; finely divided hard wood sawdust, 2 parts by volume; magnesium chloride, 22 to 26 degrees Baumé, in determinate quantity.

35 In compounding the above ingredients, the first step is to mix the asbestos with the sawdust and moisten the same with the magnesium chloride. But enough of the chloride is used to thoroughly moisten the solids without excess of liquid residue. The balance of 40 the solid ingredients are then added to the aforesaid mixture and agitated while thin with more of the magnesium chloride, so that the resulting mixture will be of a thick creamy consistency and uniform in texture. 45

50 The enamel is now ready for use.

In order to apply the novel enamel, I use a unique method whereby I may secure an even and perfect coating. Thus, I pour a thin layer of the enamel into a shallow mold having the appearance of a pan or tray. I have illustrated this mold in perspective in Figure 1 of the accompanying drawing, the bottom being indicated at 5, the wall at 6 and a reinforcing marginal flange at 7. Constructed in this manner, the mold may be formed reasonably large without becoming subject to warping or distorting tendencies, since the wall 6 and flange 7 strengthen the mold to a sufficient degree.

The depth of the mold is so dimensioned as to accommodate a sufficient layer of the enamel and provide only so much space above this layer as to accommodate the thickness of the wallboard. Thus, the height of the enamel layer is indicated in Figure 1 by the finely dotted lines, and it may be assumed that the mold is only so much higher as to receive a sheet of wallboard of standard or predetermined thickness.

Before the wallboard is laid in the mold, I span the latter near the ends with cross rails 8, each indicated in the plan view of Figure 2, then depositing the wallboard 9 upon these rails. The longitudinal section of Figure 3 also illustrates this arrangement, and it will be noted that the wallboard is marginally short of the mold walls by a narrow space.

The wallboard is now supported in close proximity to the enamel, and in order to coat the underside thereof, I place a medial cross bar 10 upon the wallboard in the position indicated by finely dotted lines in Figures 2 and 3. This cross bar is sufficiently heavy to depress the medial portion of the wallboard to the extent of dipping its under side in the enamel, as clearly indicated in Figure 4. The wallboard is, of course, sufficiently flexible to permit this action, and it may be assumed that the medial portion of the same has received a complete, transverse coating of the enamel. In order to coat the balance of the under surface of the wallboard, I work toward the ends thereof by gradually moving or shifting the outer cross rails 8 in an outward direction so as to progressively lower

the elevated portions of the wallboard into contact with the enamel. This method of coating the wallboard permits the enamel to gain upon the surface of the wallboard gradually and displace the air under the wallboard evenly, so that no air globules or pockets may be caught in the enamel to prevent the thorough coating of the same upon the surface of the wallboard. The gradual coating of the enamel thus eliminates the possibility of crust or shell-like formations in the enameled surface after the same has dried, which formations may chip or peel off to expose the original wallboard surface and defeat the purposes of my enamel.

It will thus be seen that by my gradual process of application, I am able to impart a full and uniform coating to the surface of the wallboard. Further, the nature of my mold enables the enamel to rise about the edges of the wallboard as the same has been fully lowered into the enamel, so that the edges receive the coating as well as the under surface. Each piece of wallboard is thus a finished piece all around.

In contemplating the properties of the novel enamel, the individual advantages of the ingredients were considered. Thus, the sawdust is a good filler, and has flexibility; the asbestos is also an incidental filler and has plastic properties; the magnesite is a cement bond; the silica is a void filler and strengthening agent, and it imparts a hardness to the product after it has dried as well as a white color; and the magnesium chloride is the vehicle and medium for the merging of the solids and the solution of the magnesite cement to form the resulting semi-liquid product.

When the enamel has dried it has a glass-like or vitreous finish, is waterproof and weather-proof and may be washed, scoured or otherwise cleaned without danger of damage to the finish. The coating is hard yet flexible, so that it will not check, crack or break when the wallboard is flexed, or when nails are driven near the edges to fasten the same. The texture of the enamel gives it a marked tenacity, which is evident when the wallboard is sawed or otherwise cut, such treatment being received by the enamel smoothly and without chipping or cracking in any manner. The enamel may be treated with colors and mixtures to give it a finish of imitation marble, wood graining, a stone effect or veining effects. In fact the enamel may be prepared to suit any desired condition or effect with ease without the loss of its above-enumerated properties or advantages. It will also be apparent that the ingredients I am using are relatively inexpensive, so that I am providing an enamel which may be produced at low cost and may therefore be given a wide use. Also, the use of the novel enamel need not be restricted to wallboard or similar

sheeting, but it may be used wherever a coating having a hard, yet flexible vitreous finish is desired, and where the water-proof and weather-proof properties are considered of especial value.

While I have suggested the ingredients in the proportions stated, I do not wish to be restricted to these proportions, but may decide to vary the same as I may see fit to suit different conditions. Also, the method of coating is not necessarily limited to the initial dipping of the wallboard at its medial portion; on the contrary I may deem it advisable to start dipping the wallboard from one or both ends, or from the sides, or from the corners. I do not restrict the claim to the point from where I start to dip the wallboard, but desire that the scope of my method cover the gradual dipping or lowering of the wallboard from any point in the surface thereof, my principle being to create a flow upon the wallboard from the given direction or directions whereby to coat the surface and displace the air without restriction of the same, so that no resistance is offered to the perfect coating of the surface by the enamel.

In conclusion, it may be stated that whatever variations may be made in the compounding or application of the novel enamel, as contemplated above, such changes will be to perfect and render the product susceptible to more uses, but will in no manner depart from the principle of the invention as covered in the appended claims.

I claim:—

1. The method of coating a sheet of firm material with an enamel, consisting of pouring a layer of the enamel into an open vessel, supporting the sheet in parallel relation to the surface of said layer, lowering the sheet with one portion of its area upon said layer by bending the sheet, and gradually lowering the balance of the sheet from said portion to progressively meet said layer until fully coated with the same.

2. The method of coating a sheet of firm material with an enamel, consisting of pouring a layer of the enamel into an open vessel, lowering the sheet with the medial portion of its area upon said layer, and gradually lowering the balance of the sheet from said portion to progressively meet said layer until fully coated with the same.

3. The method of coating a sheet of firm material with an enamel, consisting of pouring a layer of the enamel into an open vessel, lowering the sheet with one portion of its area intermediate its ends upon said layer, maintaining such portion depressed by the agency of a weight and gradually lowering the balance of the sheet from said portion to progressively meet said layer until fully coated with the same.

4. The method of coating a sheet of firm material with an enamel, consisting of pour-

70

75

80

85

90

100

105

110

115

120

125

130

ing a layer of enamel into an open vessel,  
lowering the sheet with a portion of its area  
intermediate its ends upon said layer, and  
gradually lowering the balance of the sheet  
from said portion to progressively meet said  
layer until the entire area and edges of the  
sheet are fully coated.

In testimony whereof I affix my signature.  
JOHN W. COWELL.

10

15

20

25

30

35

40

45

50

55

60

65